

# United States Patent [19]

Desrochers et al.

[11] Patent Number: 5,021,122

[45] Date of Patent: Jun. 4, 1991

## [54] EXPLODED BARK PRODUCTS

[75] Inventors: Michel J. Desrochers, Dollard des Ormeaux; Michel Jean, Pointe Claire; Michel P. Drouin, Ile Perrot, all of Canada

[73] Assignee: Domtar Inc., Montreal, Canada

[21] Appl. No.: 468,347

[22] Filed: Jan. 22, 1990

[51] Int. Cl.<sup>5</sup> ..... D21H 11/00

[52] U.S. Cl. ..... 162/150; 162/165;  
162/181.6

[58] Field of Search ..... 162/13, 21, 93, 225,  
162/150, 165, 181.3, 181.6, 103, 18, 10, 11, 12;  
264/124; 428/535, 537.1

## [56] References Cited

### U.S. PATENT DOCUMENTS

1,663,503 5/1928 Mason ..... 162/21  
3,984,363 10/1976 D'Alelio ..... 530/502  
4,879,066 11/1989 Crompton ..... 427/419.6

## FOREIGN PATENT DOCUMENTS

1213711 11/1986 Canada .

## OTHER PUBLICATIONS

Rydholt, Pulping Processes, Interscience Publishers, 1967, p. 100.

Primary Examiner—Richard V. Fisher

Assistant Examiner—Charles K. Friedman

Attorney, Agent, or Firm—Antoine H. Gauvin

## [57] ABSTRACT

A shaped product comprising exploded bark. Preferably the shaped product comprises exploded softwood bark having at least 23% cellulose and at least 18% lignin and polyphenols content, based upon the dry weight basis of the bark. One of the methods to make the shaped product comprises exploding softwood bark to obtain exploded softwood bark having at least 23% cellulose and at least 18% lignin and polyphenols content, compressing that exploded bark into a shaped product, while removing in part water, and drying the shaped product to remove the remaining water.

23 Claims, 1 Drawing Sheet





## EXPLODED BARK PRODUCTS

## FIELD OF THE INVENTION

This invention relates to shaped products comprising exploded bark, preferably softwood bark and most preferably softwood bark having at least 23% cellulose content and at least 18% lignin and polyphenols content, said percent being on the dry weight basis of said bark, and particularly boards of exploded barks herein-after referred to as: "exploded bark boards" and to the methods of making same, where in the bark so exploded, the cellulose content as well as the lignin and the polyphenols contents are maximized.

This invention is also directed to methods for making same as defined hereinabove, and particularly those for making exploded bark boards with or without compatible fragmented material adjuncts, and preferably boards having improved flexural strength and low water absorption as compared with conventional boards having no exploded bark.

The term "lignin and polyphenols" as referred to in the disclosure and claims is meant to refer to lignin and polyphenols, as quantitatively determined by analysis before or after exploding the bark, which means that the lignin and phenols after exploding the bark may have somewhat different chemical structures but are not degraded to low sugars.

## BACKGROUND OF THE INVENTION

Barks are generally considered wastes from commercial manufacturers.

Exploded wood is known, and so far, has been considered a curiosity rather than a tool to obtain new products having particular properties.

The prior art discloses steam explosion of wood, and also bark, but in order to extract the oils and sugars inherent to trees (wood and barks). These oils are for instance: fatty acids, fatty alcohols, fatty ketones, aromatic esters, aromatic acids, phenols and polyphenols, alkanes, alkenes. Normally oils and sugars represent about 30% of which about 15 to 20% are sugars. These sugars and phenols may be water-extracted and the oils solvent-extracted.

There is also disclosed, in Canadian Patent 1,213,711 as invented by Shen, Ku-Cheng, dated 86, 11, 12, a process for converting lignocellulosic materials into composite products whereby, as stated on Page 4, penultimate paragraph, the inventor has disclosed that free sugars can be generated from hemicellulose in any lignocellulosic materials and be utilized as a bonding agent for reconstituted composite products. The inventor converts hemicellulose into free sugars, carbohydrates or saccharides by auto-hydrolysis.

As stated on Page 6 of the patent, "First, acetic acid is formed by cleavage of acetyl side chains, and the weak acidic environment thus created is sufficient to promote hydrolysis of hemicellulose. The depolymerization reaction is believed to be a sequential reaction. During the initial phase of the reaction process, random attack by acid in hemicellulose chains produces oligomers of varying degrees of polymerization. The oligomers are further hydrolyzed to monomers which are further degraded to furfural and other decomposition products. Simultaneously, the lignin portion of lignocellulosic materials is also decomposed and hydrolyzed to low molecular weight lignin and lignin products. Only the cellulose remains relatively unchanged. The steam-

treated lignocellulosic materials normally have about 20 to 30% of water solubles which contain sugars, sugar polymers, dehydrated carbohydrates, furfural products, lignin products. The free sugars, furfural, and other decomposition products are essential parts of the present invention. When chemically transformed under heat and pressure, they would thermoset and crosslink into a polymeric substance acting as both a bonding and bulking agent for the reconstituted composite products from the steam treated lignocellulosic materials."

## BRIEF DESCRIPTION OF THE INVENTION

Broadly stated, the invention is directed to a method of making a shaped product containing exploded bark, preferably softwood bark, which comprises:

exploding bark obtain exploded bark, preferably softwood bark and most preferably softwood bark having at least 23% cellulose and at least 18% lignin polyphenols contents, compressing said exploded bark to obtain new shaped products and in part remove the water, and drying the shaped products to remove the remaining water.

In a particular embodiment, the invention is directed to the method of making a steam-exploded shaped product comprising:

steam-exploding softwood bark by steam-explosion at a temperature ranging from 150° to 210° during a period from 2 minutes, up to from 5 minutes when said temperature is about 210° C. to up to 8 minutes when said temperature is 150° C., to maximize the cellulose and lignin polyphenols contents of the bark,

removing the water while shaping said drying bark under heat and pressure in order to obtain a unitary shaped product consisting essentially of exploded softwood bark.

In a preferred embodiment the invention is directed to the method of making a shaped product containing an exploded softwood bark which comprises:

steam exploding softwood bark at a temperature from 150° C. to 210° C. during a period from 2 minutes, up to from 5 minutes when said temperature is about 210° C. to up to 8 minutes when said temperature is 150° C.

mixing wood fibers with said bark so exploded, removing in part water from the mixture of bark wood fibers, thus obtained,

compressing said mixture into a shaped product defining a board, thereby removing further water, and drying said board to remove the remaining water.

In another embodiment the invention comprises steam-exploding softwood bark as above, to obtain wet exploded bark having at least 23% cellulose content, and a water content of about 50 to 70%,

mixing from 65 to 99% by weight of wood fibers, with from 1 to 35% by weight of said wet exploded bark to obtain a highly diluted dispersion having a consistency of about 1 to 2% solid in water, laying said diluted dispersion over a perforated surface in order to obtain a layer of wood fibers and bark,

removing therefrom water until a mat is obtained, further removing water by exerting pressure and vacuum on said mat and drying said mat.

It should be noted that the 35% by weight of exploded bark could also be increased when a very high vacuum is used in order to remove the water.

The invention also comprises:

steam exploding said bark at a temperature ranging from 150° to 210° C., during a period from 2 minutes up to from 5 minutes when said temperature is about 210° C., to up to 8 minutes when said temperature is 150° C.,

mixing at least one compatible adjunct therewith and compressing said mixture into a shaped product defining a board, thereby removing further water, and drying said board to remove the remaining water.

If desired after steam exploding and before mixing, water may be removed in part from said bark so exploded.

The shaped product can take any form, molding, sheets, boards, tiles are for instance some of the species of that genus.

The drying is generally carried out to remove the remaining portion of the water to a level of about the ambient humidity, although, this is not essential.

The invention is also directed to various shaped products comprising exploded softwood bark, having at least 23% cellulose content, and at least 18% lignin and polyphenols contents, said % being on the dry weight basis of said bark.

### THE EXPLOSION

By the terms "exploded" bark, "exploding" bark and "explosion" of bark, are meant compressing with a fluid under pressure and heat, bark for a given period of time, and then abruptly releasing the pressure to obtain by "explosion" fiber-like and powder-like products, wherein the lignin and the polyphenols are spread on the surface of the fibers hereinafter referred to as "exploded bark". The conditions of temperature and duration of the explosion are set in order to maximize the cellulose, lignin and polyphenols contents as will be discussed hereinbelow and to prevent hydrolysis of hemicellulose and to prevent sugar formation and other degradation of the cellulose, lignin and polyphenols.

This process is preferably conducted by steam exploding at a temperature to open the bark while maximizing the production of cellulose. Pressurized steam is generally at a temperature between 210° and 150° C., preferably from 200 to 210° C. during 2 to 5 minutes is most preferred. Low temperatures to maximize cellulose production would be desirable, however, as the temperature is lowered below 200° C. the efficiency of the explosion of the bark to free the cellulose is reduced. Higher temperatures must be avoided, as they decrease the fiber length and degrade cellulose at the expense of non useful products as will be demonstrated hereinbelow.

In order to obtain the explosion of the bark, pressures as low as 50 psi and as high as 500 psi may be used. Preferably however, pressures of 200-300 psi or thereabout are conveniently used.

### BRIEF DESCRIPTION OF THE DRAWING

Further features, objects and advantages will be evident following detailed description of the preferred embodiments of the present invention taken in conjunction with the accompanying drawings, in which:

FIG. 1 is a graph representing the flexural strength of boards in psi (ordinate) versus the percentage by weight of exploded softwood bark (abscissa), in a board con-

taining exploded softwood bark and wood fibers as described in Examples 1, 2, 3 and Sample A.

FIG. 2 is a graph representing the flexural strength of boards in psi (ordinate) versus the percentage by weight of exploded hardwood bark (abscissa), in a board containing exploded hardwood bark and wood fibers.

### DESCRIPTION OF A PREFERRED EMBODIMENT

One of the preferred ways of carrying out the invention consists in steam exploding softwood bark at a temperature from 150 to 210° C., preferably from 200 to 210° C. during 2 to 5 minutes, to obtain a wet exploded softwood bark having at least 23% cellulose content, and a water content by weight of about 50 to 70%.

Thereafter, this wet exploded bark is mixed with from 65 to 99% by weight of wood fibers to obtain a highly diluted dispersion having a consistency of about 1 to 4%, preferably 1 to 2% solid. This consistency may also be more or less, if one desires. The wood fibers may be derived for instance from saw dust, wood shavings and the like, by digesting these shavings and/or saw dust, refining and de-fibering. The wood thus obtained in suspension can be mixed in a mixer with the wet exploded fibers. Other additives may be added, if desired.

From the mixer, the resulting mixture can be sent to a mat former having a reservoir provided partly therein with a rotatable drum, said drum having a perforated surface, whereby the mixture adheres to the perforated surface by a vacuum created inside the drum, such as with an Oliver TM filter machine. As the drum rotates a mat is formed while water is removed. The mat so obtained is then displaced over a plurality of squeezing rollers while holding the mat between endless belts. Pressures of 3 to 80 psi may be used or even higher. The mat is then heat dried to remove the water, with a COE TM steam dryer to form a slab which is cut to the desired size.

If desired, this product can be sandwiched with papers or laminated. A board containing 100% bark product obtained by steam explosion is stronger than a 100% wood fiber board, generally made under the name : "hardwood-or softwood-panels".

### OTHER WAYS OF CARRYING OUT THE INVENTION

If desired, a thermomechanical treatment in aqueous continuous phase may be conducted. In such a system the bark is suspended in an aqueous system, homogenized i.e. well mixed, pressurized, pressure released, thereby flashing out and filtered.

Although steam exploded bark is preferred, there are other ways as thermomechanical in vapour phase, using other compatible solvents in critical or supercritical phase instead of water to produce the explosion of bark. Care should be taken by one skilled in the art, when solvents are used so as to not affect the aims of this invention which is maximized cellulose formation as well as lignin formation.

Staketech which is a continuous process, as commercially available by Stake Technology Ltd., 208 Weycroft Road, Oakville, Ontario, Canada, L6K 3T8, which converts lignocellulose by continuous steam displacement under pressure as high as 450 psi: For instance, at 450 psi during 1-4 minutes.

If desired, the oils and sugars which are inherent to trees and which represent about 30% by weight of the

bark, may be removed by extraction before making a shaped product, however, this is generally less preferred because of possible loss of the low volatile materials experienced during such extractions. It may for instance be removed by steam distillation.

### SHAPING

Pressures of 3 to 80 psi and more may be used to shape the exploded bark alone or with other compatible fragmented material adjuncts. Higher pressures are 10 preferred, since at low pressures, the flexural strengths are less. The product obtained at high pressures is more water impermeable, absorbing less water.

The pressure exerted on the exploded bark is the sole ingredient that produces the unitary formation of the 15 shaped products. Yet it produces, without glues, resins or adhesives, the unitary shaped products, say a board having flexural strengths that is better than one with conventional wood fibers. The lignin on the cellulose fibers is the active ingredient that may be used to glue 20 the cellulose fibers together. Also, the dimensional stability is improved. These products may be used in areas where particle boards are generally used, and are preferred to such particle boards.

### MIXTURES CONTAINING EXPLODED BARK

Also seen above, the exploded bark could be mixed with compatible adjuncts which are fragmented material adjuncts which have no hindering effect on the purpose of the invention. As typical examples of compatible adjuncts are polymeric fragmented materials, for instance phenolic foam i.e. fully cross-linked or other foams if desired. Polyethylene, polyesters and other polymers could also be used. Also inorganic fragmented materials are contemplated, for instance gypsum (for instance 1 to 10% by weight of the board), cement, and the like. The exploded bark can be mixed with cement into moldable products, for instance, in an amount ranging from 10 to 50% by weight of the board.

The exploded bark could also be mixed with wood 40 pulp using conventional methods, whether virgin or recycled (for instance 5-20%) to be shaped into a ply for a carton i.e. liver board and corrugated medium, in the making of boxes. The exploded bark could also be shaped into a ply in the making of interior or exterior plywood. It could also be mixed with 60 to 90% wood 45 pulp to make other useful products. Low density panels as is well known having 0.16 to 0.42 g/cm<sup>3</sup> or 9.99 to 26.22 lb/ft<sup>3</sup>. Medium density panels having 0.53 to 0.80 g/cm<sup>3</sup> or 33.09 to 49.94 lb/ft<sup>3</sup> and high density panels 50 higher to said 0.8 g/cm<sup>3</sup> or 50 lb/ft<sup>3</sup> may be produced by exerting the necessary pressure when compressing into a shaped product.

The exploded bark could also be used for making interior ceiling felt, roofing felt, interior and exterior 55 sheathings, as well as for composite materials that are either laminated or molded.

The exploded softwood bark could also be mixed with hardwood bark, but in a preferred embodiment in an amount ranging from 1 to 35% of hardwood bark 60 having a more preferably cellulose content of at least 11%.

Also exploded hardwood barks could be used with wood fibers for making panels.

### OTHER TREATMENTS

It has also been found that a surface treatment, such as a quick treatment with 1% H<sub>2</sub>O<sub>2</sub>, NaOH or H<sub>2</sub>SO<sub>4</sub>,

produces improved properties of the shaped product comprising exploded bark, such as flexural strength, dimensional stability, water absorption.

After explosion, the exploded bark can be used as 5 such or treated as follows:

- (a) with oxidizing agents, for instance peroxides;
- (b) with a solvent to remove oils and other oil soluble products;
- (c) as in (b) followed by a treatment as in (a);
- (d) with a Lewis base, for instance NaOH, KOH;
- (e) as in (b) followed by (d);
- (f) with a solvent to remove sugars;
- (g) with a Lewis acid, such as sulfuric, acetic, hydro chloric.

For the above steps (a) to (g) the exploded barks are generally treated in an aqueous suspension for about 5 minutes to half an hour.

The exploded bark board could also be made by drying and then heat pressing the exploded bark, for instance at 3 psi during 5 minutes after vacuum filtration. The time and pressure can be extended, for pressures as high as 80 psi and more could be used.

### EXAMPLES

25 The following examples will serve to illustrate in detail, particular embodiments of the invention.

#### EXAMPLES 1 TO 10

Various exploded bark boards (examples 1 to 10) 30 were made as described under "Description of a preferred embodiment" hereinabove, with softwood fibers (WF), softwood bark (EB) steam exploded at 210° C. during 2 minutes and phenolic foam (PF) in various amounts, using pressures of about 3 psi.

As seen in Table 1, the dimensional stability, (Dimensional stab) in thickness (T), width (W) and the length (L) of the boards were evaluated at 90° C., 10% humidity during two weeks. The same order of results were obtained under a 50% humidity at 20° C., and 95% humidity at 30° C.

Also as shown in Table 2, the dimensional stability of the board was measured after 3 weeks at a temperature of 30° C. under a 95% humidity.

Table 3 illustrates the dimensional stability obtained after 3 weeks at 90° C. and 10% humidity.

In each case as shown in Table where conditions are closer to normal conditions, 2 and 3, the dimensional stability is as good as or better than Sample A which is a standard fiberboard. Sample B has a PF:EB:WF ratio of 0:0:100 and is a commercially available fiberboard.

The density (D) of the boards in (lb/cu.ft) was obtained after the drying of the panels. The water absorption (Absorp.) was measured after submerging the panels in water at 25° C. for 2 hours, then the panels were left on a table for  $\frac{1}{2}$  hour at room temperature under normal humidity conditions prior to measuring their weights as per ASTM-C209. As can be seen, the density increases with the addition of exploded bark, while the water absorption decreases.

TABLE 1

| Example | PF:EB:WF | Dimensional Stability |      |      | D<br>lb/ft <sup>3</sup> | Water Absorp.<br>% Volume |
|---------|----------|-----------------------|------|------|-------------------------|---------------------------|
|         |          | T %                   | W %  | L %  |                         |                           |
| 1       | 0:10:90  | 3.79                  | 0.27 | 0.08 | 19.27                   | 14.28                     |
| 2       | 0:20:80  | 1.60                  | 0.18 | 0.26 | 20.15                   | 19.56                     |
| 3       | 0:40:60  | 0.00                  | 0.24 | 0.21 | 21.96                   | 12.33                     |
| 4       | 0:80:20  | 0.06                  | 0.01 | 0.20 | 24.87                   | 7.86                      |
| 5       | 20:60:20 | 0.35                  | 0.10 | 0.42 | 22.24                   | 10.02                     |

TABLE 1-continued

| Example  | PF:EB:WF | Dimensional Stability |      |      | D<br>lb/ft <sup>3</sup> | Water Absorp.<br>% Volume |
|----------|----------|-----------------------|------|------|-------------------------|---------------------------|
|          |          | T %                   | W %  | L %  |                         |                           |
| 6        | 10:60:30 | 0.05                  | 0.04 | 0.04 | 21.91                   | 15.06                     |
| 7        | 10:40:60 | 0.15                  | 0.13 | 0.27 | 20.27                   | 14.47                     |
| 8        | 20:40:60 | 0.40                  | 0.09 | 0.03 | 20.08                   | 7.72                      |
| 9        | 20:70:50 | 1.34                  | 0.00 | 0.28 | 20.05                   | 12.08                     |
| 10       | 20:30:50 | 0.08                  | 0.30 | 0.47 | 19.22                   | 9.95                      |
| Sample A | 0:0:100  | 0.20                  | 0.05 | 0.16 | 16.84                   | 16.49                     |

TABLE 2

| Example   | Dimensional stability |      |      |
|-----------|-----------------------|------|------|
|           | T %                   | W %  | L %  |
| 1         | 5.80                  | 0.42 | 0.42 |
| 2         | 6.06                  | 0.48 | 0.48 |
| 3         | 4.19                  | 0.25 | 0.28 |
| 5         | 1.87                  | 0.60 | 0.38 |
| 6         | 3.09                  | 0.27 | 0.36 |
| 7         | 4.05                  | 0.51 | 0.54 |
| 8         | 2.10                  | 0.35 | 0.37 |
| 9         | 2.40                  | 0.69 | 0.86 |
| 10        | 3.22                  | 0.31 | 0.27 |
| Sample A  | 6.88                  | 0.97 | 0.57 |
| Sample B* | 5.27                  | 0.38 | 0.20 |

(\*Conventional panel)

TABLE 3

| Example  | Dimensional stability |      |      |
|----------|-----------------------|------|------|
|          | T %                   | W %  | L %  |
| 1        | 3.30                  | 0.47 | 0.38 |
| 2        | 3.24                  | 0.52 | 0.44 |
| 3        | 2.21                  | 0.42 | 0.53 |
| 4        | 1.74                  | 0.58 | 0.50 |
| 5        | 1.89                  | 0.53 | 0.85 |
| 6        | 2.60                  | 0.48 | 0.48 |
| 7        | 2.69                  | 0.50 | 0.44 |
| 8        | 2.53                  | 0.36 | 0.41 |
| 9        | 2.33                  | 0.33 | 0.46 |
| 10       | 3.00                  | 0.58 | 0.45 |
| Sample A | 3.82                  | 0.46 | 0.43 |

The thermal resistivity (R) and the permeability (PERM) were also determined for some of the boards made as shown in Table 4.

TABLE 4

| PF:EB:WF | R    | PERM.  |
|----------|------|--------|
| 0:50:50  | 2.55 | 48.00  |
| 20:43:47 | 2.60 | 115.00 |

45

50

TABLE 4-continued

| PF:EB:WF | R    | PERM. |
|----------|------|-------|
| Sample A | 2.62 | 61.00 |

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1010

1015

1020

1025

1030

1035

1040

1045

1050

1055

1060

1065

1070

1075

1080

1085

1090

1095

1100

TABLE 7

|                                                                                   | Starting Material | Example 20 Residue | Example 21 Residue | Example 22 Residue | Example 23 Residue | Sample E or 24 Residue |
|-----------------------------------------------------------------------------------|-------------------|--------------------|--------------------|--------------------|--------------------|------------------------|
| Temperature of steam explosion                                                    | —                 | (130° C.)          | (140° C.)          | (150° C.)          | (180° C.)          | (210° C.)              |
| Time in minutes                                                                   | —                 | 2                  | 2                  | 2                  | 2                  | 2                      |
| Part of residue dissolved in water containing sugars following washing with water | —                 | 25                 | 24                 | 26                 | 47                 | 67.0                   |
| Lignin (NaOH) and Polyphenols                                                     | 30                | 27                 | 27                 | 26                 | 19.5               | 14.2                   |
| Cellulose                                                                         | 31.9              | 27.7               | 22.3               | 31.1               | 14.9               | 10.9                   |
| Pentosanes                                                                        | 14                | 12                 | 10                 | 6                  | 7                  | 2                      |

\*(in % by weight based upon the weight of the starting material on a dry basis) (— not carried out)

### EXAMPLES 20 TO 24

The same was repeated as in Examples 16 to 19 and Sample D but using hardwood bark. The results shown in Table 7 were obtained. As is easily seen the steam explosion in the case of hardwood bark must be between 130° and 160° to maximize the cellulose, the lignin and the polyphenols content. However, as one skilled in the art knows, the lignin of hardwood bark and of softwood bark are chemically different.

Having described the invention, modifications will be evident of those skilled in the art without departing from the spirit of the invention, as defined in the appended claims.

As a result boards were made as in Example 1-3 but with hardwood bark, steam exploded at 210° C. during 2 minutes and the results are tabulated of FIG. 2 which clearly demonstrates the significant advantage of softwood exploded bark. However steam exploded hardwood bark can be successfully used within some limit in combination with softwood exploded bark to make wood fiber boards.

### EXAMPLES 25 TO 36

Various exploded bark boards were made with softwood fibers (WF), softwood bark steam exploded (EB) and in some cases (Examples 29 to 36 inclusive) with phenolic foam (PF) as a compatible fragmented adjunct. The flexural strengths (FS) of boards is for: in psi were measured, and the percentage increase of flexural strength calculated in comparison with 25 which is a sample.

Results are shown in Table 8

TABLE 8

| Example   | EB:WF    | FS  | % increase in FS |
|-----------|----------|-----|------------------|
| Sample 25 | 0:100    | 231 | 0                |
| 26        | 10:90    | 306 | 40               |
| 27        | 20:80    | 355 | 54               |
| 28        | 40:60    | 492 | 113              |
| Example   | PF EB WF | FS  | % increase in FS |
| 29        | 20:40:60 | 235 | 2                |
| 30        | 20:60:20 | 298 | 29               |
| 31        | 20:30:50 | 313 | 35               |
| 32        | 20:43:37 | 231 | 0                |
| 33        | 14:50:36 | 287 | 24               |
| 34        | 10:60:30 | 298 | 29               |
| 35        | 9:36:55  | 300 | 30               |
| Sample 36 | 0:0:100  | 231 | 0                |

Having described the invention, numerous modifications will be evident to those skilled in the art without departing from the spirit of the invention, as defined in the appended claims.

The invention claimed is:

- 20 1. A pressed and dried shaped product comprising at least 7.5% of exploded softwood bark having at least 23% cellulose and at least 18% lignin and polyphenols content said percent being on the dry weight basis of said bark said product being held together by no other binder than the adhesives present in said exploded bark, the lignin on the cellulose being the active ingredient to 25 glue the cellulose fibers together.
2. The shaped product as defined in claim 1 wherein said exploded bark is steam exploded bark.
3. The shaped product as defined in claim 1, being a steam-exploded bark board.
- 30 4. The steam-exploded bark board as defined in claim 3, consisting essentially of pressed, dried, steam exploded bark.
- 35 5. The steam-exploded bark board as defined in claim 3, comprising a mixture of steam-exploded softwood bark and at least one compatible fragmented adjunct.
- 40 6. The steam-exploded bark board as defined in claim 5, wherein said adjunct is wood fiber.
7. The steam-exploded bark board as defined in claim 5, wherein said adjunct is a fully cross-linked phenolic foam.
- 45 8. The steam-exploded bark board as defined in claim 5 wherein said adjunct is from 1 to 35% of a steam-exploded hardwood bark having at least 11% cellulose content.
9. The steam-exploded bark board as defined in claim 3, wherein said steam-exploded bark board is from a steam-exploded bark treated with a member selected from the group consisting of Lewis acids, Lewis bases and oxidizing agents.
- 50 10. The steam-exploded bark board as defined in claim 3, wherein said bark the oils inherent to trees have been substantially removed.
11. The steam-exploded bark board as defined in claim 3, wherein said bark contains the oils inherent to trees.
- 55 12. The steam-exploded bark board as defined in claim 6, wherein said adjunct of wood fiber is essentially of softwood fibers.
13. The steam-exploded bark board as defined in claim 6, wherein said adjunct of wood fiber is of a mixture of hardwood - softwood fibers.
- 60 14. The steam-exploded bark board as defined in claim 12 being a low density fiber board having a density from 11 lb/ft<sup>3</sup> to 30 lb/ft<sup>3</sup> and a flexural strength from 300 to 500 psi.
- 65 15. The board as defined in claim 5, wherein said adjunct is gypsum in an amount ranging from 1 to 10% by weight of the board.

**11**

16. The board as defined in claim 5, wherein said adjunct is cement in an amount ranging from 10 to 50% by weight of the board.

17. The shaped product as defined in claim 1, consisting of exploded softwood bark in an amount ranging from 2 to 20% by weight and from 80 to 98% of wood pulp shaped into a ply for a liner board and corrugating medium.

18. The shaped product as defined in claim 1, consisting of 1 to 40% of steam-exploded softwood bark and 60 to 99% of wood pulp shaped into a ply for a plywood, based upon the weight of said plywood.

19. The exploded bark as defined in claim 1 consisting of said exploded softwood bark and a polymer.

**12**

20. The steam-exploded bark board as defined in claim 12 wherein said cellulose is in the form of fibers that are surrounded with said lignin and said polyphenols and glued therein.

5 21. The shaped product as defined in claim 1 wherein said cellulose is in the form of fibers that are surrounded with said lignin and said polyphenols and glued therein.

10 22. The steam-exploded bark board as defined in claim 12 being a medium density fiber board having a density from 33 to 50 lb/ft<sup>3</sup> and a flexural strength greater than 500 psi.

23. A shaped product as defined in claim 1 comprising hardwood exploded bark.

\* \* \* \* \*

15

20

25

30

35

40

45

50

55

60

65